

# United States Patent [19]

Wright et al.

[11] Patent Number: 4,867,644

[45] Date of Patent: Sep. 19, 1989

[54] COMPOSITE MEMBER, UNITARY ROTOR MEMBER INCLUDING SAME, AND METHOD OF MAKING

[75] Inventors: E. Scott Wright, Mesa; James G. Kenehan, Phoenix, both of Ariz.

[73] Assignee: Allied-Signal Inc., Morris Township, Morris County, N.J.

[21] Appl. No.: 51,000

[22] Filed: May 15, 1987

[51] Int. Cl.<sup>4</sup> F01D 5/28

[52] U.S. Cl. 416/230; 416/241 R; 428/660; 501/35

[58] Field of Search 416/229 R, 229 A, 230 R, 416/230 A, 241 R, 244 R; 428/660, 608; 420/419; 501/35; 29/156.8 R; 74/572; 164/97

## [56] References Cited

### U.S. PATENT DOCUMENTS

- |           |         |                    |           |
|-----------|---------|--------------------|-----------|
| 2,757,901 | 8/1956  | McVeigh            | 416/244 R |
| 3,554,667 | 1/1971  | Wagle              | 416/218   |
| 3,554,668 | 1/1971  | Wagle              | 416/218   |
| 3,610,777 | 10/1971 | Wagle              | 416/198   |
| 3,625,634 | 12/1971 | Stedfeld           | 416/198   |
| 3,649,425 | 3/1972  | Alexander          | 428/660 X |
| 3,656,864 | 4/1972  | Wagle              | 416/190   |
| 3,711,936 | 1/1973  | Athey et al.       | 416/230 X |
| 3,717,443 | 2/1973  | McMurray et al.    | 428/660 X |
| 3,765,796 | 10/1973 | Stargardter et al. | 416/244 R |
| 3,787,141 | 1/1974  | Walsh              | 416/244 R |
| 3,813,185 | 5/1974  | Bouiller et al.    | 416/198   |

- |           |         |                 |             |
|-----------|---------|-----------------|-------------|
| 3,904,316 | 9/1975  | Clingman et al. | 416/218     |
| 3,966,523 | 6/1976  | Jakobsen et al. | 156/159     |
| 3,973,875 | 8/1976  | Bird            | 416/241 B   |
| 4,011,295 | 3/1977  | Tree et al.     | 416/241 B X |
| 4,076,456 | 2/1978  | Tree et al.     | 416/241 B   |
| 4,096,615 | 6/1978  | Cross           | 29/156.8 R  |
| 4,132,828 | 1/1979  | Nakamura et al. | 428/608 X   |
| 4,152,816 | 5/1979  | Ewing et al.    | 29/156.8 R  |
| 4,363,602 | 12/1982 | Martin          | 416/230 R   |
| 4,465,434 | 8/1984  | Rourk           | 416/230 R   |
| 4,506,721 | 3/1985  | Ban et al.      | 164/97      |
| 4,570,316 | 2/1986  | Sakamaki et al. | 416/241 B X |
| 4,697,324 | 10/1987 | Grant et al.    | 29/419 R    |

## FOREIGN PATENT DOCUMENTS

- 1040697 10/1953 France  
976237 11/1964 United Kingdom

Primary Examiner—Robert E. Garrett  
Assistant Examiner—Joseph M. Pitko  
Attorney, Agent, or Firm—Terry L. Miller; James W. McFarland

## [57] ABSTRACT

A composite member includes circumferentially extending ceramic fibers in a metallic matrix. A rotor member integrally includes such a ceramic fiber/metal matrix composite member to reinforce a homogeneous remainder portion of the rotor member with respect to centrifugally induced stresses. Method of making are included in the disclosure.

21 Claims, 2 Drawing Sheets





FIG. 1

FIG. 2



FIG. 3

24

24

28

24

FIG. 5



FIG. 4

FIG. 5



FIG. 7

FIG. 6



FIG. 8



FIG. 9

70-72



FIG. 10

**COMPOSITE MEMBER, UNITARY ROTOR MEMBER INCLUDING SAME, AND METHOD OF MAKING**

**BACKGROUND OF THE INVENTION**

The field of the present invention is composite ceramic filament/metal matrix members. More particularly, the present invention relates to rotor members for gas turbine engines having composite ceramic filament/metal matrix portions therein. Such a unitary rotor member includes an integral reinforcing portion defined by such a ceramic filament/metal matrix composite member. Still more particularly, the present invention relates to a method of making a ceramic filament/metal matrix composite hoop member. A method of making a unitary member including such a composite ceramic filament/metal matrix hoop reinforcing portion is also disclosed.

Conventional methods of making filament reinforced polymer matrix composite rings is disclosed in U.S. Pat. 3,966,523 to Jakobsen et al, issued 29 June 1976. The Jakobsen teaching provides a filament reinforced polymer matrix ring which is intended to remain a separate reinforcing component. Similar conventional teachings are set forth in U.S. Pat. Nos. 3,765,796 and 3,787,141 wherein rotor members for turbine engines are shown to include fiber reinforced composite reinforcing rings. These reinforcing rings are received within annular cavities of the turbine engine rotor member and receive centrifugally induced stresses upon relative radial growth of the metallic components of the rotor member. Although the reinforcing hoop members of composite material may be captured within the rotor member, they remain separate component parts which are subject to relative rotation and vibrational imbalances.

It is understood in the pertinent art that the high tensile strength provided by fiber reinforced composite materials may advantageously be employed to sustain centrifugally induced tangential stresses within a high speed rotor member. However, as is illustrated by the above-outlined conventional teachings, the fiber reinforced composite member has always been considered as a separate reinforcing component which must be supported and restrained within a rotor member of a turbine engine. Such a separate reinforcing component presents many problems with respect to its restraint and support prior to its assuming its full function as a reinforcing member. That is, the metallic components of the rotor member will experience much greater radial growth in response to centrifugally induced stresses than does the composite member. In order to best utilize such a composite reinforcing hoop, it is therefore required that the metallic components be allowed to sustain a considerable portion of the centrifugally induced stresses and to undergo such radial growth before additional centrifugally induced stresses are transferred to the composite reinforcing hoop member. Thus, prior to the time of assuming its full reinforcing function, the composite hoop member is somewhat free to assume non-concentric positions with respect to the rotational axis of the rotor member. Of course, should the composite reinforcing member deviate significantly from the rotational axis of the rotor member, very significant vibrational forces are sure to result.

An additional aspect of such conventional teachings is that only radially outwardly directed forces may be transferred to the composite member by contact be-

tween annular surfaces at the inner bore of the composite hoop member and annular surfaces at an inner wall of the metallic components of the rotor member. Consequently, the metallic components of the rotor member must be designed to sustain significant radially-directed tensile stresses in order to transfer the centrifugally induced tangential stresses to the inner wall portion of the metallic components. Of course, such a design inexorably results in the metallic components of the rotor member being heavier than desired.

**SUMMARY OF THE INVENTION**

In view of the above, it is an object of the present invention to provide a composite ceramic fiber/metal matrix hoop member wherein the metal matrix of the hoop member is capable of metallurgical integration with the metallic components of a rotor member of a gas turbine engine.

An additional object of the present invention is to provide a unitary rotor member for a gas turbine engine having a composite ceramic fiber/metal matrix reinforcing portion integral therewith.

An additional object of the present invention is to provide a method of making a composite metal matrix ceramic fiber reinforcing hoop member as described above.

An additional object of the present invention is to provide a method of making a unitary rotor member for a combustion turbine engine wherein an integral portion of the rotor member is defined by a ceramic fiber/metal matrix hoop member.

The present invention provides a composite ceramic fiber/metal matrix member wherein a plurality of circumferentially extending ceramic fibers are each continuous circumferentially through at least 300 degrees of arc, and the metal matrix is continuous circumferentially, radially, and axially. That is, the metal matrix is continuous, or monolithic, throughout the entire extent of the composite member.

The present invention further provides unitary or truly one piece, metallic rotor member including as an integral portion thereof, a composite ceramic fiber/metal matrix member as described above. The metal matrix of the composite member is continuous with the metal of the remainder of the rotor member so that the latter is truly of integral metallic continuum, and includes an integral portion having ceramic fibrous reinforcement therein.

Further to the above, the present invention provides a method of making a composite ceramic fiber/metal matrix member including the steps of winding a unidirectional mat of ceramic fibers, laminating the fiber mat with metallic foil, interbonding the foil and ceramic fiber mat, slitting the bonded foil and fiber mat into elongate ribbons, winding the ribbons into a hoop form, consolidating the wound ribbon hoop form into a unitary body, and forming the consolidated unitary body into a determined shape.

The present invention also provides a method of making a unitary or one piece rotor member for a combustion turbine engine having as an integral part thereof a ceramic fiber/metal matrix composite member, and including the steps of forming a composite member as outlined above and further including the additional steps of providing rotor member monolithic components cooperatively defining a cavity of determined shape, assembling the rotor member monolithic compo-

nents with a composite hoop member having the determined shape captively received in the cavity, consolidating the rotor member monolithic components and the composite hoop member into a unitary body, and further preparing the rotor member for utilization in a combustion turbine engine.

An advantage of the present invention resides in the consolidation of the fibrous reinforcing filaments with the metallic matrix of the composite reinforcing member. That is, the plural fibrous reinforcing members are embedded in the metal matrix in mechanical bonding relationship therewith such that the metal and ceramic fibers are effectively a unitary body. A further advantage of the present invention resides in the unitary nature of a rotor member including a ceramic fiber/metal matrix composite member as outlined above. Such a rotor member advantageously enjoys a continuous metal matrix throughout the member, that is, the metal matrix of the composite is continuous with the monolithic or integral metallic structure of the remainder of the rotor member such that discontinuities and stress concentrations as would be created by conventional constructions are effectively avoided by the present invention. Additionally, because the metallic infrastructure of the rotor member is substantially continuous, centrifugally induced stresses within the rotor member may be transferred to the composite portion thereof by shear and tensile stresses along the radially extending and radially outer axial extents thereof as well as by radially directed compressive forces received adjacent the bore of the composite member. In summary then, a rotor member incorporating a composite member according to the invention enjoys much superior stress transfer to the composite reinforcing hoop and much better utilization of the available strength of the materials of construction than do the best of the known technologies outlined above.

Additional objects and advantages of the present invention will appear from a careful reading of the following detailed description of a single preferred embodiment of the invention taken in conjunction with the following drawing figures.

#### BRIEF DESCRIPTION OF THE DRAWING FIGURES

FIG. 1 depicts a fragmentary cross-sectional view of an elongate unidirectional ceramic fiber mat and a pair of elongate metallic foils in preparation to lamination thereof into a unitary body;

FIG. 2 depicts a fragmentary cross-sectional view of an elongate composite ceramic fiber/metal matrix ribbon resulting from consolidation of the lamina depicted in FIG. 1;

FIG. 3 shows a fragmentary cross-sectional view of a hoop form resulting from winding onto a mandrel multiple layers of ribbon as depicted in FIG. 2;

FIG. 4 is a perspective view of a hoop form composed of multiple layers of ceramic fiber/metal matrix ribbon as described above, and a closed exterior sheet metal can completely enclosing the would ribbon hoop form preparatory to HIP processing;

FIG. 5 depicts a fragmentary cross-sectional view of a ceramic fiber/metal hoop form of FIG. 4 and after HIP processing thereof;

FIGS. 6 and 7 show a perspective view and a cross-sectional view, respectively, of a finished ceramic fiber/metal matrix composite member;

FIG. 8 depicts a fragmentary cross-sectional view of a ceramic fiber/metal matrix member as depicted in FIGS. 6 and 7, received within a cavity defined cooperatively by a pair of metallic rotor member parts;

FIG. 9 shows an axial cross-sectional view of a unitary metallic rotor member including as an integral reinforcing portion thereof a ceramic fiber/metal matrix composite; and

FIG. 10 shows steps in the method of making a ceramic fiber/metal matrix composite member, and a monolithic rotor member integrally including such a composite reinforcing member, according to the invention.

#### DETAILED DESCRIPTION OF THE PREFERRED EMBODIMENT

FIG. 1 depicts a fragmentary cross-sectional view of a unidirectional elongate ceramic fiber mat 10 disposed between a pair of elongate metallic foils 12 and 14 preparatory to lamination of the foils and the ceramic fiber mat. That is, both the mat 10 and foils 12, 14 are elongate both perpendicular to the plane of FIG. 1, and laterally. Even though only 6 fibers 16 are shown in FIG. 1, it will be understood that the mat itself contains multiple fibers and preferably is constituted of approximately 130 substantially parallel fibers 16 per inch of width. Each of the fibers 16 is substantially identical and includes a central carbon monofilament core 18 having a diameter of about 0.0013 inch. The core 18 is surrounded by a layer of chemical vapor deposited (CVD) beta silicone carbide 20. Covering the layer 20 of beta silicone carbide is an extremely thin carbon-rich layer 22 having a graded silicone content. By way of example, the layer 22 is preferably only 3 to 4 microns thick and is provided for the purpose of inhibiting high temperature reactivity between the beta silicone carbide layer 20 and the metallic foils 12 and 14. Overall, the filaments 16 have an outer diameter of about 0.0056 inch. Such fibers display a tensile strength of about 550 KSI, a Young's modulus of about 58 PSI ( $\times 10^6$ ), and a density of about 0.11 pound/in<sup>3</sup>. A fiber which has been found to be acceptable for this invention is available from Avco Corporation, and is identified as SCS-6 silicon carbide fiber. The metallic foils themselves are composed of a titanium alloy Ti-6A1-4V.

According to the preferred embodiment, the unidirectional fiber mat 10 is constructed by winding onto a large drum multiple substantially parallel wraps of the ceramic fibers 16. That is, the wraps of elongate fiber 50 traverse axially across the drum helically from near one edge thereof to adjacent the other drum edge. An acrylic binder is applied to the drum surface and to the fibers to hold the latter in place after winding. Following curing of the acrylic layer, the fibers and acrylic 55 binder are separated from the drum surface intact as a unidirectional mat. For example, a single axial cut may be made across all of the fiber wraps so that the elongate fibers and acrylic binder are peeled from the drum surface intact as a single sheet. This sheet or mat of acrylic binder and ceramic fibers is then placed between the metallic foils 12 and 14, sealed in a vacuum bag, and press diffusion bonded to form ceramic fiber-metal matrix sheet material. During such press diffusion bonding, the interior of the vacuum bag is evacuated and the 60 temperature increased to about 1000° F. As a result, the acrylic binder is decomposed entirely into gaseous and/or volatile decomposition products, and is removed by the partial vacuum. Subsequently, a combination of

pressure, temperature and time are employed to consolidate the foils 12, 14 and the fibers 16 into a unitary body. By way of example, a pressure of from 6000 (6KSI) to 10,000 (10 KSI) and a temperature of from 1650° F. to 1750° F., maintained for a time period of from 20 minutes to 45 minutes has proven to be sufficient to interbond the foils 12, 14 into a unitary body with the fibers 16.

Viewing now FIG. 2, it will be seen that the resulting ceramic fiber/metal matrix sheet material 24 is composed of approximately 35 percent by volume of fiber 16 with the remainder being constituted by metallic matrix 26. The metallic matrix is composed of the metallic foils 12 and 14 which are metallurgically united by the vacuum diffusion pressing process such that they are integrally interbonded. Even though only a very small transverse section of the sheet material 24 is depicted, in fact, the sheet 24 has a width including several hundreds of the fibers 16 and may be ten feet or more in length. A convenient way of utilizing the sheet material 24 involves making a series of parallel cuts therein, with each cut parallel to the fibers 16. Consequently, each successive cut separates a ribbon-like length of the sheet material 24 from the remainder thereof. The width of the ribbon is selected to match its intended use.

Turning now to FIG. 3, it is seen that an annular hoop form 28 is composed of multiple wraps of ceramic fiber/metal matrix sheet material as depicted in FIG. 2. The sheet material 24 is employed in the form of elongate ribbon produced as described above. The lengths of ribbon may conveniently be wound spirally upon a mandrel (not shown) such that each length of ribbon provides several complete wraps around the mandrel. Consequently, the elongate fibers 16 extend through at least 360 degrees of arc. By way of example, the sheet material 24 may be made by using a winding drum of about four foot diameter. As a result, the sheet material and ribbon has a length of about 12 feet. The outer diameter of hoop form 28 is about 8 inches. Each wrap of hoop form 28 will then require no more than 2 feet of ribbon. Thus, it may be expected that the elongate fibers 16 extend spirally within the hoop form at least 6 complete wraps. The width of the ribbon is equal to that of the hoop form 28 so that wraps of ribbon extend spirally outwardly, but no traversing of the ribbon is necessary in building up the hoop form. Again, in the annular hoop form 28 the overall fiber content is approximately 35 percent by volume with the remainder being defined by the metallic matrix 26.

FIG. 4 depicts an annular hoop form 28 as depicted in FIG. 3 having an annular closed metallic can in surrounding relationship therewith. The annular can includes a radially inner annular axially extending portion 32 and a similar radially outer annular axially extending portion 34. The portions 32 and 34 are connected by a pair of axially spaced apart radially extending portions 36 and 38. All of the portions 30, 32, 34 and 36 are sealingly interconnected with one another to define a closed annular metallic can surrounding and receiving the annular hoop form 28 previously described.

Following "canning" of the annular hoop form 28 as is depicted by FIG. 4, the resulting assembly is subjected to hot isostatic pressing (HIP) processing to consolidate both the ceramic fiber/metal matrix ribbons 24 of the annular hoop form and the exterior metallic can itself. As a result, a unitary body is formed which is fragmentarily depicted in cross-section in FIG. 5. It is seen in FIG. 5 that the individual discrete ribbons 24 are

now integrally interbonded to form a continuous metal matrix having a multitude of circumferentially extending ceramic fibers received therein. Again the bulk of the resulting annular ceramic fiber/metal matrix body is composed of about 35 percent by volume of the ceramic fiber 16 with the remainder being defined by the metal matrix.

FIGS. 6 and 7 in conjunction depict a resulting composite ceramic fiber/metal matrix member which is formed by machining the consolidated body described above. That is, after HIP processing of the canned assembly depicted in FIG. 4, the resulting body appears very much similar to that depicted in FIG. 4 with the exception that the metal matrix is continuous throughout the body and the ceramic fibers are integrally received therein. It will be seen that the annular composite body 44 illustrated in FIGS. 6 and 7 is generally frustoconical in configuration, and includes a plurality of circumferentially extending ceramic fibers 16. The annular body includes an axially extending radially outer surface 46 and a pair of axially spaced apart generally frustoconical radially extending end surfaces 48 and 50. The annular body 44 also defines an axially extending through bore 52.

Turning now to FIG. 8, it will be seen that a disk-like rotor member workpiece 54 is composed of a pair of somewhat similar homogeneous metallic rotor member components 56 and 58 which cooperatively define a recess 60 matching in shape the annular composite ceramic fiber/metal matrix member 44. The components 56, 58 are made of titanium alloy Ti-6Al-2Sn-4Zr-2Mo (Ti-6242). The annular composite body 44 is received within the cavity 60 such that a pair of boss portions 62 and 64, respectively, of the components 56 and 58 extend into and substantially fill the bore portion 52 of the composite body 44. The rotor member components 56 and 58 also cooperatively define an interface surface 66 extending radially outwardly from the cavity 60 to the radially outer peripheral surfaces 68 and 70 of the components 56 and 58. A circumferentially continuous sealing weld 72 is applied at the junction of the surface 66 with the radially outer peripheral surfaces 68 and 70 to sealingly unite the component pieces 56 and 58 with the composite body 44 captively received within the cavity 60.

The assembly depicted in FIG. 8 is subsequently subjected to hot isostatic pressing (HIP) processing to metallurgically unite the components 56 and 58 and the composite body 44. Consequently, the HIP processed workpiece is subjected to further machining operations to result in a substantially completed rotor member 74 as is depicted in FIG. 9. The rotor member 74 defines an axially extending throughbore 76 extending through the bore portion 52 of the composite body 44. The rotor member 74 also is metallurgically continuous to include the metallic matrix of the composite body 44. That is, the metallic material of rotor member 44 is metallurgically integral with the metallic matrix of composite body 44 at the surface of bore 52, at the end surfaces 48 and 50 of the composite body, and at the radially outer surface 46 of the composite body. In point of fact, these surfaces cease to exist after HIP processing of the assembly depicted in FIG. 8. Therefore, the rotor member 44 may be considered to be composed of a continuous metallic matrix or infrastructure having a portion reinforced by circumferentially extending and circumferentially continuous ceramic fibers 16. Further consideration of the completed rotor member will reveal

that the metal matrix of the composite portion 44 and the substantially homogeneous metallic structure of the components 56, 58 cooperate after HIP processing to define a metallic infrastructure which is continuous throughout the rotor member 74. That is, considered, radially axially, or circumferentially, the metallic structure of rotor member 74 is continuous. Further, the rotor member 74 is free of voids or cavities. At the radially outer peripheral surface (now referenced with the combined reference numerals used previously) 70-72 of rotor member 74, a bladed ring may be attached, or structural features may be provided to carry individual compressor blades, for example.

FIG. 10 summarizes the steps in the method of making both the composite body 44, which has been described previously, and the rotor member 74 integrally including such a composite body such as is depicted in FIG. 9. As set forth in FIG. 10, it will be seen that first of all a unidirectional fiber mat is provided by winding ceramic fibers, for example, onto the surface of a drum. The resulting unidirectional fiber mat is laminated with metallic titanium foil and the resulting laminated foil and fiber mat are subsequently consolidated by vacuum diffusion pressing, a species of HIP processing. The resulting composite ceramic fiber/metal matrix foil is then slit into ribbon-like pieces. The ribbons are subsequently wound onto a mandrel to define a composite ceramic fiber/metal matrix hoop form. Such a hoop form is then canned in a closed sheet metal can which is metallurgically compatible with the metallic matrix of the hoop form, and the completed canned assembly is consolidated by HIP processing. Finally, the consolidated canned hoop form is subjected to machining to define a desired outer configuration for the resulting annular composite body. In order to further utilize the resulting annular composite body, rotor member homogeneous monolithic metallic components are provided which define a cavity of the same shape as the annular composite body. An annular composite body is subsequently assembled with the monolithic metallic components of the rotor member and sealed therein such that subsequent HIP processing metallurgically unites the metallic matrix of the composite body with the monolithic metallic components. Final machining of the unitary body resulting from HIP processing then provides a unitary rotor member having an integral reinforcing portion thereof of ceramic fiber/metallic matrix composite.

Having depicted and described our invention by reference to a particularly preferred embodiment thereof with sufficient detail and information provided to allow one ordinarily skilled in the pertinent art to make and use the invention, it is our desire to protect our invention in accord with applicable law. While the invention has been described by reference to a particularly preferred embodiment thereof, such reference does not imply a limitation upon the invention and no such limitation is to be inferred. The invention is to be limited only by the spirit and scope of the appended claims which also provide additional disclosure and definition of the invention.

We claim:

1. Apparatus comprising a disk-like unitary rotor member having an integral composite ceramic fiber/metal matrix portion reinforcing a homogeneous metallic remainder portion thereof, said rotor member defining a metallic infrastructure which is continuous axially, radially, and circumferentially therewithin and which

includes both said metal matrix of said composite portion and said homogeneous metallic portion, said rotor member further being substantially free of internal voids. said composite ceramic fiber/metal matrix portion including a plurality of circumferentially extending ceramic fibers, each one of said ceramic fibers comprising a central monofilament core, and a layer of beta silicon carbide ceramic surrounding said core.

2. The invention of claim 1 wherein each one of said plurality of ceramic fibers also comprises an outer carbon-rich layer having a graded silicon content.

3. The invention of claim 2 wherein said ceramic fibers are Avco SCS-6 silicon carbide fiber.

4. The invention of claim 1 wherein said metal matrix of said composite ceramic fiber/metal matrix portion comprises titanium alloy Ti-6AL-4V.

5. The invention of claim 1 wherein said homogeneous metallic remainder portion comprises titanium alloy Ti-6AL-2SN-4Zr-2Mo(Yi-6242).

6. The invention of claim 1 wherein said composite ceramic fiber/metal matrix portion comprises substantially 35% by volume of ceramic fibers.

7. Apparatus comprising a disk-like unitary rotor member integrally including an annular composite ceramic fiber/metal matrix portion, said annular composite portion defining a through bore having a radially inwardly disposed interface surface, a pair of axially spaced apart annular end surfaces each extending radially outwardly of said through bore, and an axially extending radially outwardly disposed outer annular surface interconnecting said pair of end surfaces, a substantially homogeneous metallic portion enclosing said annular composite portion; said metallic portion metallurgically interbonding with said annular composite portion in stress-transmitting relation at each of said interface surface, said pair of end surfaces, and said outer surface.

8. The invention of claim 7 wherein said metal matrix part of said annular composite ceramic fiber/metal matrix portion, and said substantially homogeneous metallic portion cooperate to define a metallic infrastructure for said rotor member, said metallic infrastructure being continuous axially, radially, and circumferentially throughout said rotor member.

9. The invention of claim 8 wherein said rotor member is further free of internal voids.

10. The invention of claim 7 wherein said annular composite ceramic fiber/metal matrix portion comprises a circumferentially extending plurality of spaced apart ceramic fibers each oriented substantially tangentially with respect to a rotational axis of said rotor member.

11. The invention of claim 10 wherein said annular composite portion comprises substantially 35% by volume of said ceramic fiber.

12. The invention of claim 10 wherein said ceramic fibers comprise a carbon monofilament core.

13. The invention of claim 12 wherein said core is substantially 0.0013 inch in diameter.

14. The invention of claim 12 wherein said ceramic fiber further includes a layer of beta silicon carbide surrounding said core.

15. The invention of claim 14 wherein said ceramic fiber further includes an outer carbon-rich layer having a graded silicon content.

16. The invention of claim 15 wherein said outer carbon-rich layer is of substantially 3 to 4 microns thick.

17. The invention of claim 16 wherein said ceramic fiber defines an outer diameter of about 0.0056 inch.

18. The invention of claim 7 wherein said ceramic fiber comprises Avco SCS-6 silicon carbide fiber.

19. The invention of claim 7 wherein said annular composite ceramic fiber/metal matrix portion comprises a metallic matrix of titanium alloy Ti-6AL-4V.

20. The invention of claim 7 wherein said substantially homogeneous metallic portion comprises titanium alloy Ti-6242.

21. A unitary disk-like rotor member comprising a substantially homogeneous metallic portion, and a com-

posite ceramic fiber/metal matrix portion enveloped completely within and reinforcing said metallic portion with respect to centrifugally-induced stresses said matrix portion including a circumferentially extending ceramic fiber having a monofilament core, said metallic portion and said metallic matrix of said composite ceramic fiber/metal matrix portion metallurgically interbonding and cooperatively defining a metallic infrastructure for said rotor member, which metallic infrastructure is continuous between said portions.

\* \* \* \* \*

15

20

25

30

35

40

45

50

55

60

65